

June 21, 1932.

R. W. STIMSON ET AL

1,863,642

MANUFACTURE OF ALLOYS

Filed March 13, 1925

Fig.1.



Fig.2.



Fig.3.



Fig.4.



*INVENTOR*  
Robert W. Stimson  
Wilhelm Borchers

BY

*Sol Shappirio*  
ATTORNEY

## UNITED STATES PATENT OFFICE

ROBERT WICKERSHAM STIMSON, OF NEW YORK, N. Y., AND WILHELM BORCHERS, OF AACHEN, GERMANY

## MANUFACTURE OF ALLOYS

Application filed March 13, 1925, Serial No. 15,2394, and in Great Britain November 6, 1924.

This invention relates to the manufacture of alloys of the type in which any number of the metalloids silicon titanium and zirconium are united with any number of miscible metallic elements, e. g., cobalt copper chromium iron manganese molybdenum nickel tantalum thorium tungsten uranium and vanadium—the chief object being to produce the alloys by means of a new or improved "direct reduction process" wherein the metallic components may be extracted with the use of carbonaceous deoxidants from sources hitherto regarded as impracticable and unprofitable i. e., metalliferous slags by-products and non-commercial aggregates of compounds and ores, although the invention is equally applicable to and includes the use of commercial ores, metalliferous concentrates aggregates of compounds and oxygenous metallic compounds. A "direct reduction process" as will be understood is one in which all components of the metallic product are extracted from a mixture of reducible materials containing different metals and in the case of the present invention it is one in which the metalloid and metallic elements are concurrently extracted from a mixture which includes reducible matter comprising compounds of any number of the metalloids silicon titanium and zirconium and reducible matter comprising compounds of metals that are miscible with them.

Carbon aluminium and silicon are reducing agents generally used in the art. Of these carbon is the least expensive and most efficient but ferruginous alloys extracted in its presence absorb percentages of carbon approximating those of cast irons and come within the grade known as "ferro alloys" or "alloy cast irons" consequently other reagents are employed when the object is to directly produce "special steels" or "alloy steels" having carbon-contents that are below 2.20% of the aggregates.

The invention is specifically directed to production of alloys of the type defined in the first preceding paragraph that contain more than 1.00% of any number of the specified metalloids and come within the low-carbon or steel grade defined in the latter preced-

ing paragraph which alloys will henceforth be designated and understood in this specification and appendant claims as the "specified alloys".

Since it is impracticable to reduce materials comprising oxygen compounds of non-ferrous metallic elements (e. g. chromite) with carbonaceous matter when the purpose is to directly recover low-carbon alloys aluminium or silicon containing reducing agents are generally used and in mass production it has been found that aluminium seldom recovers more than 70% also that silicon rarely extracts more than 40% of the non-ferrous metal contained in ores whereas metallic yields effected with carbonaceous reagents usually exceed 90% of the aggregate. Therefore to minimize metal-losses occasioned by use of aluminium or silicon it is customary to mix ore with slags emerging from the reactions and include such mixtures of metalliferous materials in subsequent furnace charges to be reduced by carbonaceous matter whereby the metal is substantially reclaimed but in a high-carbon state. It is to be observed from the foregoing that only a portion of the metal obtainable from ores of non-ferrous metals is extracted in the form of low-carbon products.

That silicon, titanium and zirconium have the property of decreasing the dissolving power of ferruginous alloys for carbon has long been known and we have now discovered how to amplify and augment the deoxidizing power of carbon when it is smelted with oxygen compounds of these elements. Through the instrumentality of the invention the "specified alloys" may be directly produced whilst smelting a mixture of appropriate reducible materials with carbonaceous matter without adding more carbon to the metallic products than is found after dissolving for example high grade ferro-silicon in alloy steels.

The invention is largely based upon disclosures resulting from experiments conducted with the view of employing slags and other metalliferous refuse as sources from which to extract metallic elements in a low-carbon state and particularly metals such as

chromium which form carbides that are stable and it may be solid at ordinary steel-making temperatures. Briefly stated, the experiments disclosed the following law regarding the "specified alloys"; the selection of fluxes and the quantities in which they are added during the melts have far-reaching influences upon (a) the quantities of silicon titanium and zirconium that may be extracted through the agency of carbon (b) the carbon contents of the metallic products and (c) the amounts of independent thermal energy that must be applied to start and accomplish the extraction reaction. To express it in another way, it was found that varying quantities of metal were extracted from equal quantities of the same materials and under like conditions as regards the application and consumption of independent thermal energy when different fluxes had been used to enhance the liquid properties of slags. It was later discovered that certain constant relations exist between the chemical compositions of final slags on the one hand and the quantities of materials that were metallified also the amounts of independent heat that were absorbed in accomplishing reactions on the other hand and we have now found how these relations or principles may be advantageously used in the art.

Three important principles disclosed by the above mentioned experiments and others directed to extracting larger quantities of silicon titanium and zirconium from their oxygen compounds are (1) that the final slag should possess neither a strongly basic nor a strongly acidic character; (2) that the predominant basic component of the final slag should itself possess only a mild instead of a strong basic chemical character, and (3) that conditions (1) and (2) should co-exist.

We have found that the preponderating basic component of final slags should be alumina with which may be associated lime magnesia and other basic oxides. And while the essential basic flux may consist of commercially pure alumina it is advantageous to employ natural aluminous matter such as corundum bauxite clays and feldspar and particularly aluminous slags from other metallurgical operations also ores or aggregates containing oxygen compounds of desired metallic elements and gangue that is rich in alumina and silica.

More specifically stated experiments directed to production of the "specified alloys" by concurrently extracting the components from a mixture of their oxides have established the following natural laws:—

(1) If alumina is reckoned as a basic oxide larger quantities of silicon titanium and zirconium are extracted from furnace charges that yield basic final slags than from otherwise equivalent charges that yield acid final slags.

(2) As regards silicon titanium and zirconium neither the quantities which are extracted under conditions that produce intensely basic final slags nor the quantities which are extracted under conditions that produce powerful acid final slags are as large as the quantities which are extracted under conditions that produce slightly basic and weak acid final slags.

(3) The chemical compositions of slags as regards non-reducible compounds have greater influence than their chemical properties upon the quantities of silicon titanium and zirconium that may be recovered by the metallurgical reduction of their oxides. Variations occur in the quantities of these elements that are extracted under conditions that form mild acid neutral and mild basic final slags other conditions being equivalent but in cases where lime is a minor instead of the predominating basic component of mild acid mild basic and neutral final slags the metallurgical recoveries are invariably larger.

(4) The largest recoveries of silicon titanium and zirconium are accompanied by final slags in which the following conditions co-exist: (a) the chemical equivalents of silica exceed the sum of the equivalents of other acidic components, and (b) the sum of the chemical equivalents of alumina lime and magnesia is not less than 75% of the equivalents of silica, while (c) the chemical equivalents of alumina are not less than 85% of the sum of the equivalents of lime and magnesia.

(5) When contained in a limy basic slag a certain proportion of alumina relinquishes its basic chemical character and becomes weakly acidic in its action the quantity being that which will neutralize the more powerful bases lime and magnesia. In these circumstances and to the extent imposed by the excess of powerful bases to be neutralized alumina must be recognized as a weak acid oxide. Alumina in excess of the quantity required to cause a state of equilibrium between acids and bases may be reckoned upon as being mildly basic.

(6) The presence of silicates (or it may be titanates or zirconates) of lime and magnesia in an aggregation of reacting materials is far less favorable to the reduction of uncombined silica (or oxides of titanium and zirconium) than alumina-silicates (or alumina-titanates or alumina-zirconates) and especially alumina itself and effect the quantitative recovery of silicon (or titanium or zirconium) accordingly.

(7) In the interest of economy furnace charges should contain silica in sufficient excess of the quantity required for the purpose of yielding silicon as to cause it to be the largest acid component of final slags but the chance presence of minor quantities of boric titanic zirconic and the like mild acid oxides

has no apparent influence upon the quantity of silicon that will be recovered and these mild acid oxides are readily neutralized by alumina.

(8) Titanium and zirconium are extracted when their oxides replace at least that quantity of silica which is employed according to the invention for the purpose of yielding silicon and by means of these substitutions titanium-containing and zirconium-containing alloys are obtained which possess influences and relations in respect to carbon sulphur and oxygen similar to those of silicon and silicon-containing alloys.

(9) When contained in acid slags that are rich in silica boric titanic and zirconic oxides are transferred from weak acids into mild bases substantially to the same extent as and for a purpose similar to that of alumina, as set forth in the above article (5), although the transition and subsequent properties are the reverse. In these circumstances therefore and to an extent prescribed by the excess of silica to be neutralized boric titanic and zirconic oxides are mildly basic while quantities exceeding those needed to cause a state of neutrality between acids and bases resume or continue with their naturally acid chemical characters.

(10) The previously listed miscible metals readily dissolve and unite with silicon titanium and zirconium when they are concurrently extracted from a mixture of materials containing their oxygen compounds and because of the generally higher mean specific gravities alloyed silicon titanium and zirconium readily sink through the slags and collect in the form of metal-baths.

According to the present invention the natural laws outlined above are applied in a direct reduction process of manufacturing the "specified alloys" and it is to be particularly observed that in contradistinction to previous proposals lime is not the principal basic component of our final slags. Dr. W. Borchers on page 565 of his "Elektrometallurgie", 3rd edition, (1903) states that low-carbon alloys containing silicon and metallic elements are obtainable by smelting oxides of the metals and silica with carbonaceous reducing agents in an electric furnace. Such processes however are wasteful as regards recoverable metallic elements and thermal energy if an attempt be made to produce metal having a silicon-content in excess of 9% of the aggregate. Whereas by means of our present process alloys containing more than 9% of any number of the metalloids silicon titanium and zirconium may be produced economically as regards independent thermal energy—a further accomplishment being that substantially all recoverable metallic elements contained in the furnace charges are extracted and recovered with the metalloids.

It is to be understood that in the following illustrative plan of operating the process materials comprising or containing the corresponding compounds of titanium and zirconium may be employed in place of the silica and silicates to be reduced and to simplify descriptions henceforth only compounds of silicon will be mentioned the purpose and intent being that the references apply to and include the corresponding compounds of titanium and zirconium.

In carrying the invention into practice we may employ any suitable type or kind of furnace (e. g. an electric furnace) which preferably has a carbonaceous hearth and smelt therein a charge comprising (a)—silica with which may be included appropriate silicates (b)—materials comprising reducible compounds of miscible metallic elements (c)—carbonaceous reducing agents and (d)—fluxes that are selected and proportioned in relation to other non-reactive, i. e. earthy matter in the furnace charge so that a final slag in accordance with the principles mentioned in the above list of articles, particularly article (4), will emerge from the reaction. The furnace preferably contains a small quantity of molten aluminous non-metallic matter such as slag from the preceding heat so that the new charge may sink into it and thereby become protected from the atmosphere. Preferably the charge is agglutinated into lumps or briquettes of a size that is most suitable for expeditious charging, its ingredients having been crushed or ground and intimately mixed together and by using pitch tar mineral oil sugar-carbon or other adhesive carbonaceous matter as a portion of the required reducing agent it also serves as a binding agent or agglutinant to hold the reactive materials in contact with each other. Independent thermal energy is applied to the charge to start and accomplish chemical reactions. When ebullition caused by escaping gases has almost ceased we may add a liquefying flux for example fluorspar borax and acid oxides such as silica also increase the bath temperature and intermittently feed small quantities of carbonaceous matter upon the slag until it becomes gray in color thus indicating that it is in a non-oxidizing and demetallized state.

As to sources from which to obtain the previously enumerated miscible metallic elements we have found and it follows from the above listed principles that provided the selection and proportional use of fluxing matter is closely observed satisfactory results may be obtained whether the sources of metallic elements be commercial ores or low-grade aggregations containing a metalliferous compound or slags and by-products containing oxygenous compounds of the desired metallic elements.

About proportioning carbonaceous reduc-

ing agents they may be used in considerable excess of theoretical requirements as indicated by the reaction equations without fear of the usual quantity of carbon finding its way into the metal-bath. The low-carbon state of the "specified alloys" when produced according to the invention may be ascribed to two causes it having been found that: (I)—use of a given quantity of carbonaceous reagent is followed by unusually large recoveries of the metalloids silicon titanium and zirconium and (II)—a portion of the metalloids is extracted from their oxygen compounds through the agency of aluminum in a nascent state. As regards cause (I):—(a)—in addition to taking better advantage of the well known properties of the metalloids in respect to carbon further significance of the increased quantities of silicon titanium and zirconium recoverable with a given quantity of carbonaceous deoxidant are (b)—a greater proportion of carbon is actually employed for reaction purposes according to the present process and (c)—the high temperature essential to a liquid aluminum slag enhances the oxidation of carbon at the expense of its inclination to combine with metallic elements while the influence of high temperature upon silicon for example is not identical. As regards cause (II):—since it has been determined that a portion of the silicon titanium and zirconium is extracted by means of aluminum a probable result of mass action is that part of the carbon which otherwise would form metallic carbides is consumed in reducing alumina also when hot nascent aluminum reacts with for example silica aluminum rather than carbon is in the immediate presence of the metallified element.

As regards final slags emerging from the reactions it is to be particularly noted that except for insignificant quantities of aluminum that may either escape in a vaporized state or enter the metal-bath no aluminum departs from the assemblage of reacting materials and slag and at the end of a melt substantially the same quantity of alumina is to be found in the final slag that was initially present in or added to the furnace charge. This is not the case with silica however for not only is silicon added to the metal-bath but at the prevailing temperature minor quantities of silicon burn in the atmosphere at the upper surface of the slag and form a gaseous compound with sulphur in which state it also escapes to the atmosphere. Final slags therefore comprise an excellent flux for employment in subsequent melts and require little treatment other than additions of the required quantities of appropriate metalliferous material and silica, which may be employed in any number of forms such as carbonaceous compounds and silicious slags, by products and aggregates of compounds, also

natural materials such as sand, quartz, quartzite and ores having a gangue that is rich in silica.

Although our invention consists mainly in the production of the "specified alloys" under conditions herein disclosed we are aware that similar alloys have been produced through the agency of other processes and we do not therefore regard the products as novel per se except when they are produced by our process.

The invention has been subjected to numerous practical applications and among them we have found that:—

(a) Alloys such as iron-cobalt-nickel-silicon, iron-chromium-molybdenum-tungsten-silicon, iron-manganese-zirconium-silicon and like quaternary and more complex alloys containing silicon and any number of the previously listed metallic elements may be produced in a low-carbon homogeneous state by smelting an intimately mixed charge consisting of ores speisses mattes and the like (that have been roasted dead if they contain objectionable volatile elements, for example, arsenic and sulphur) silicious material carbonaceous reducing agents and fluxes so proportioned that they will unite with other non-reducible matter in the furnace charge and form a final slag as hereinbefore described and defined.

(b) Cupro-silicon alloys such as the deoxidants used in the production of copper, alloys containing copper and castings made therefrom are readily and cheaply produced by this process. It is preferred to prepare a receptive non-metallic bath by melting a natural alumino-silicate such as clay or an aluminous slag from a previous operation into which we feed a briquetted mixture of silica carbonaceous matter and fluxing matter as hereinbefore defined. The silica-carbon-flux briquettes are then covered with a briquetted reactive mixture consisting of copper oxide carbonaceous matter and fluxes as hereinbefore described (in other test cleaned copper turnings or scrap was substituted for the copper oxide briquettes). Because of its specific gravity liquid copper emerging from the reacting materials or it may be the molten copper scrap slowly descends through the silica-carbon reacting mixture and becomes dissolved in or absorbs en route (see article (10) above) silicon which because of its low specific gravity is slowly moving upward. In this united state the copper-silicon alloy has a specific gravity that causes it to descend through the slag and accumulate in a metal-bath which is formed thereunder.

(c) Ores and other materials containing the previously listed metallic elements which, after being subjected to beneficiation or benefaction treatment, find little use in the art because of undesirable metallic inclusions or objectionable metalloidal impurities indirect-

- ly constitute a good source from which to recover their metals by means of this process. For example prepared or beneficiated phosphorous-containing manganese ores that are 5 plentiful in Brazil and elsewhere where smelted with carbonaceous matter and suitable fluxes but the usual chemical and thermal practices were reversed (i. e., we used acid instead of basic practice and avoided 10 the strong reducing conditions and high temperature that favour the extraction of manganese from its oxide) with the result that iron and phosphorous oxides were reduced, whilst the manganese oxide with practically 15 no phosphorous and only a portion of the iron oxide passed into, or were absorbed by and retained in the non-metallic accessory product, or slag. In this way a slag was produced which contained a greater ratio of 20 manganese to iron than is usually found in the better grades of manganese ores. This non-metallic accessory product was then subjected to the metallifying process herein disclosed whereby a manganese-iron-silicon alloy was produced that was exceedingly pure 25 and rich in manganese also a final slag that was exceptionally free from metals and therefore particularly adapted to use in the manufacture of cement and artificial stone. 30 Moreover the high-phosphorous cast iron that was extracted from the manganese ore was purified by means of basic open-hearth practice whereby refined carbon steel and a valuable highly phosphorated fertilizing 35 slag were produced.
- (d) A further and particularly useful application of the invention consists in making it serve as part of an improved cyclic process for the economical production of ferruginous alloys that contain one or more of the 40 alloy elements cobalt chromium manganese molybdenum nickel titanium tungsten uranium and the like which alloys have combined carbon and silicon contents amounting to less than 2.20% also combined phosphorous and 45 sulphur contents amounting to less than 0.50% of the aggregates. It is known in the art that in order to produce alloys of this class by direct ore reduction processes the oxygen-containing metalliferous materials from 50 which the metallic components are extracted must be employed in such excess over theoretical requirements as to produce (by reaction with a low-carbon reducing agent, e. g. 55 silicon) slags that are very rich in metallic elements and hitherto the presence of so much metal in slags has constituted a loss.
- By means of the invention however substantially all metallic elements except aluminum 60 calcium and magnesium are extracted from the slags. Therefore in the production of alloys defined in the last preceding paragraph we employ an abundance of oxygen-containing metalliferous materials for two 65 essential purposes: first, for the purpose of providing a sufficient quantity of metalliferous materials to react with silicon during the extraction reaction (the reaction being started and accomplished by the application of independent thermal energy as differentiated 70 from exo-thermically evolved heat) and, second, to provide a liberal excess of unreduced metallic oxides to purify the metal-bath during and after reaction with the solid reducing agent i. e., to oxidize and remove undesirable 75 quantities of silicon and carbon that inevitably pass into the metal-bath whenever a silicon-alloy reducing agent is used. In fact for these two purposes we employ the metalliferous material to an excess which is generally regarded as economically impracticable and thereby expedite reactions. Instead of being wasteful this practice according to the invention merely increases the means of effecting economy because the non-metallic accessory products or slags which are rich in metallic elements are subjected to reduction action in what will be designated the first step of the process whereby their metals are recovered in the form of silicon-alloys 80 that are employed in the second step to react with and extract recoverable metals from ores or other suitable metalliferous materials. 85
- To illustrate procedure according to the invention we cite the production of an iron-chromium-silicon alloy and its use as a reducing agent in the production of chromium alloys of all types and grades it being understood that the furnace practice may be augmented abbreviated or otherwise altered as occasion and expediency demand and that other alloy elements may be included when their presence is desired:— 90
- First, preferably we employ an electric furnace having a carbonaceous hearth and lining in which is smelted a charge consisting of:—(a) a chromium-containing slag either together with or without chromite; (b) a suitable source of silicon as silica; (c) any 100 suitable carbonaceous matter preferably in excess of the quantity required to complete reaction, and (d) fluxes which are selected and proportioned in relation to the earthy matter in other components of the charge so 105 that a final slag as hereinbefore defined, particularly in article (4), will emerge from the reduction reaction. The metallic product is an iron-chromium-silicon alloy which is to become the reducing agent that is employed 110 in the second step of the process while the slag that is produced therewith is especially adapted to the requirements of the cement and kindred industries. 115
- Second, we use another direct arc electric furnace in this step, which has a non-carbonaceous hearth and lining—it being understood that in cases wherein the reaction is caused to occur over a steel or ferruginous metal-bath for the purpose of adding the ex- 120 125 130

tracted metal to it the physical state and chemical composition of the metal-bath as regards phosphorus sulphur silicon and carbon will be suitable for the purpose in view. The iron-chromium-silicon alloy produced in the first step of the process is brought into and maintained in reaction with chromite or a chromium compound by the continuous application of independent thermal energy the reducible chromium-containing material preferably being employed in such excess over requirements that less than 40.0% of the chromium contained therein will be recovered. Obviously this excess may be diminished when the intent is to add silicon to the extracted metals. Suitable and sufficient fluxes such as lime fluorspar and borax are employed with and added to the above mentioned reactive materials and when desired the reaction is caused to occur above a metal-bath which may be covered with the customary shallow non-oxidizing calcareous protective blanket while the quantity of chromium which it is desired to add to the metal-bath determines the quantities of iron-chromium-silicon reducing agent and chromite to be employed. As a result of this reaction and practice we produce refined chromium alloy steel together with a slag that is rich in chromium; and, finally, we use this chromium-containing slag in a repetition of the first step or operation thus rendering the process cyclic. The outstanding feature of the second step is the employment of so much reducible, i. e., metalliferous material that 60.0% or more of the oxides contained therein will pass into or remain in the slag instead of being reduced.

In order to provide a lively reaction in the second step of the process the iron-chromium-silicon reducing agent preferably has a silicon-content in excess of 15.0% of the aggregate. The process includes the employment of more than one reducing agent as required by the complexity of the metal being produced; thus we may use iron-chromium-silicon, iron-molybdenum-silicon and like iron-silicon alloys to react in conjunction with ores or compounds of chromium in the second, i. e. the reduction alloying and refining step of the process.

The process further includes the employment at appropriate times of suitable metallic enriching bath-additions also degasifying and deoxidizing bath-additions and slags as required.

The following specific example is cited to illustrate one manner of operating the process it being understood that no commitments and limitations are implied as regards either details of procedure, such for example, as the method of preparing a suitable metalliferous material for further treatment and the furnace practice, or the proportional use of materials, or the type and kind of furnace that may be used also that the invention may

be otherwise employed in processes of producing "the specified alloys" within the scope of the herewith appended claims.

This heat was run in a direct-arc furnace having a carbonaceous hearth (laid over heat insulating material) and graphitized carbon electrodes as it was desired that the electrodes should be composed of material that was reducing in its chemical relation to the furnace charge. Thus particles dropping from the electrodes augmented the supply of reducing agents but obviously it is economically inadvisable to permit carbon electrodes to come into physical contact with the furnace charge, once the arcs are struck, until the metal-yielding oxygenous compounds have been substantially reduced.

A chromiferous material, of a grade that is too low to find use in commerce, was prepared for further treatment by being crushed only, as the purpose was to determine the value of its direct metallic product. Otherwise it would have been washed, and, according to a frequently important but not essential feature of the invention, preparatorily smelted under conditions that would extract iron in part whilst largely fluxing its chromic oxide into the slag which would then be subjected to further treatment. An analysis of the chromiferous mineral indicated:—  
17.38%—Cr; 9.92%—Fe; 11.33%—SiO<sub>2</sub>; 31.94%—Al<sub>2</sub>O<sub>3</sub>; 0.96%—CaO, and 14.12%—MgO, which for the purpose of easy calculation was charted according to the chemical equivalents, thus:—

#### Gram-equivalents

| In 1000 g. ore                          | Equiv. weights | Basic | Acid | C for reduction |
|-----------------------------------------|----------------|-------|------|-----------------|
| Cr 173.8 g.                             | 17.3           |       |      | 10              |
| Fe 99.2 g.                              | 28             |       |      | 3.54            |
| SiO <sub>2</sub> 113.3 g.               | 15             |       |      |                 |
| Al <sub>2</sub> O <sub>3</sub> 319.4 g. | 18.79          |       | 7.5  |                 |
| CaO 9.6 g.                              | 28             | 0.34  |      |                 |
| MgO 141.2 g.                            | 20             | 7.05  |      |                 |
|                                         |                | 26.18 | 7.5  |                 |

The amounts of chromiferous mineral, quartz, aluminous flux (which was slag from a previous heat) and lime, were calculated according to the "oxygen ratio" to form a sesqui-silicate final slag of the characteristic composition set forth in the previous list of articles particularly in article (4) a sufficient surplus of silica being included to add over 25% of silicon to the metal-bath. In this particular case the following ratios of reactive materials were employed, namely 1000 units of chromite, 764 units of quartz, and 453 units of carbonaceous matter. Obviously the surplus of silica will be increased when the object is to produce an alloy that is richer in silicon and correspondingly lower in carbon; however it had already been found that relatively small quantities of met-

als such as were contained in the chromiferous mineral to be reduced could be almost completely recovered by means of the invention when they were concurrently extracted 5 with about 25% silicon.

The carbonaceous matter (in this heat consisting of petroleum coke and tar) was calculated to provide an excess of about 50% over the theoretical requirements, it having 10 been found that a seeming extravagant excess causes a more lively reaction without adding carbon to the metal-bath also it decreases the consumption of electrodes and minimizes destruction of the carbonaceous furnace hearth 15 and lower side walls.

The reactive materials were ground, intimately mixed and agglutinated into briquettes, of a size that expedited charging, through the agency of tar.

20 It is not imperative to use more than one composition when briquetting the reactive materials however it should not be overlooked that the specific gravity of silicon is considerably lower than that of titanium and less 25 than half that of zirconium and the tendency of silicon to separate, rise to the surface of the slag and burn in the atmosphere is not small. It is preferred therefore to include no metalliferous material in a portion of the 30 briquettes.

Furnace practice used in the heat, cited by way of illustration, was as follows: the arcs were struck on some aluminous slag which had been shovelled into the pre-heated furnace and when it was molten briquettes containing no ore were intermittently fed in, followed by briquettes containing ore. High power input was applied as soon as possible the furnace was luted to check the escape of 40 heat and the furnace charge was eventually controlled at a temperature of about 1700°-1750° C. The liquidity of the slag was adjusted as required by means of silica fluor-spar and borax additions; and, when a sample 45 of the slag indicated by its light gray color and otherwise that it was substantially demetalized, powdered coke was added the electrodes were lowered into the slag for a few minutes and the current readjusted to 50 produce a hot tapping temperature.

Because of the last carbon addition the final slag was medium grey in color, it was dense, it contained 0.58%—Cr<sub>2</sub>O<sub>3</sub> and 0.46%—FeO and had the following chemical constitu- 55 tion:

Gram-equivalents

| In 1000 g. slag                         | Equiv. weights | Basic | Acid | Equalizer |
|-----------------------------------------|----------------|-------|------|-----------|
| SiO <sub>2</sub> 176.3 g.               | 15             | 11.7  | 22.4 |           |
| Al <sub>2</sub> O <sub>3</sub> 380.5 g. | 17             |       |      |           |
| CaO 297.5 g.                            | 28             | 10.6  |      |           |
| MgO 125.4 g.                            | 20             | 6.2   |      |           |
|                                         |                | 16.8  | 11.7 | 22.4      |

The chemical constitution of the final alloy was:

|                       | Per cent |
|-----------------------|----------|
| Silicon               | 24.60    |
| Chromium              | 43.20    |
| Carbon                | 0.40     |
| Iron (not determined) | 31.80    |

while its physical structure is shown in the accompanying micrographs, in which:

Figures 1 and 2 are two different micrographs of the structure as shown by etching with concentrated hydro-chloric nitric acids and magnifying 100 diameters.

Figure 3 is a micrograph as shown by etching with picric acid and magnifying 100 diameters.

Figure 4 is a micrograph of a portion of the structure shown in Figure 3 but magnified 800 diameters.

By the terms "chemical equivalents" and "equivalents" it will be understood that we mean the combining weights which are the molecular weight divided by the valency. It will further be understood that the word "lime" is meant to embrace both of the fluxing materials—limestone and quicklime.

What we claim is:

1. In a process of manufacturing the specified alloys which comprehends extracting metalline and metallic elements from a mixture of reducible matter comprising compounds of any number of the metalloids, silicon, titanium and zirconium and reducible matter comprising compounds of any number of miscible metals with a reducing agent the step of adding fluxing matter to the furnace charge whose chemical relations to other constituents of the furnace charge are such that a final slag is produced which is neither strongly basic nor strongly acidic whilst its principal basic component has only a mild basic character.

2. In a process of manufacturing the specified alloys which comprehends extracting metalline and metallic elements from a mixture of reducible matter comprising compounds of any number of the metalloids, silicon, titanium and zirconium and reducible matter comprising compounds of any number of miscible metals and a carbonaceous reducing agent, the step of adding fluxing matter with and to the furnace charge in such proportions that a final slag is produced in which the following conditions co-exist:—(a) the chemical equivalents of silica are not less than the sum of the equivalents of other acid compounds and (b) the sum of the chemical equivalents of alumina lime and magnesia is not less than 75% of the equivalents of silica whilst (c) the chemical equivalents of alumina are not less than 85% of the sum of the equivalents of lime and magnesia.

3. In a process of manufacturing the specified alloys which comprehends extract-

ing metalline and metallic elements from a mixture of reducible matter comprising compounds of any number of the metalloids, silicon, titanium and zirconium and reducible matter comprising compounds of any number of miscible metals, also a reducing agent and fluxing matter and wherein a final slag is produced in which the following conditions co-exist:—(a) the chemical equivalents of silica are not less than the sum of equivalents of other acid components and (b) the sum of the chemical equivalents of alumina, lime and magnesia is not less than 75% of the equivalents of silica, whilst (c) the chemical equivalents of alumina are not less than 85% of the sum of the equivalents of lime and magnesia, the step of employing any number of metalliferous slags, by-products and aggregates of compounds as a source from which to obtain a miscible metal.

4. In a process as set forth in claim 1, the step of applying independent thermal energy to the furnace charge.

5. In a process as set forth in claim 1, the step of feeding the reactive materials into a bath of aluminous non-metallic matter.

6. In a process as set forth in claim 1, the step of employing alumina as the preponderant basic slag forming component of the furnace charge.

7. In a process as set forth in claim 1, the step of employing alumina as the preponderant basic slag forming component of the furnace charge, with associated smaller quantities of magnesia and lime.

8. In a process as set forth in claim 1, the step of employing any number of carbonaceous agglutinants to cause the ground and intimately mixed reactive materials to adhere together.

9. In a process as set forth in claim 1, the step of employing any number of carbonaceous reducing agents.

10. In a process as set forth in claim 1, the step of employing any number of reducing agents in any excess of quantities required according to the chemical equations of the reduction reactions.

11. In a process as set forth in claim 3, the step of employing any number of carbonaceous reducing agents in any excess of quantities required according to the chemical equations of the reduction reactions.

12. In a process as set forth in claim 3, the step of providing metalliferous slags, by-products and refuse for further and reduction treatment which comprehends reducing metalliferous material under conditions favorable to an oxide of one metal being substantially metallified whilst an oxygenous compound of another metal that is miscible with any number of the metalloids, silicon, titanium and zirconium is not readily metallified and becomes embodied in the non-metallic accessory product.

13. In a process as set forth in claim 3, the step of preparing metalliferous slags, by-products and refuse for further and reduction treatment which comprises reducing metalliferous material under chemical and thermal conditions that are favorable to the reduction of an oxid of iron whilst being unfavorable to the ready extraction of a non-ferrous metal.

14. In a process as set forth in claim 3, wherein metalliferous slags, by-products and refuse are provided for further and reduction treatment, the step of applying independent thermal energy to the reactive materials whereby an oxid of one metal is readily metallified whilst an oxygenous compound of another metal that is miscible with any number of the metalloids, silicon, titanium and zirconium is not readily metallified and becomes embodied in the non-metallic accessory product.

15. In a process as set forth in claim 3, wherein metalliferous slags, by-products and refuse are prepared for further and reduction treatment, the step of employing acid furnace practice under conditions that are favorable to the reduction of an oxid of one metal whilst being unfavorable to the extraction of a non-ferrous metal that is miscible with any number of the metalloids silicon, titanium and zirconium.

16. A process as set forth in claim 3, carried out under conditions that favor the extraction of objectionable metalloids and undesirable metals and otherwise resist their passage into or absorption and retained in the slag, and thereafter subjecting the slag to reduction by means of carbonaceous reducing agents while applying independent thermal energy thereto.

17. In a process as set forth in claim 3, wherein manganiferous slags and by-products are prepared for further and reduction treatment by the reduction of manganiferous materials, the step of employing temperatures that are high enough to cause the extraction of phosphorus and low enough to be unfavorable to the reduction of the oxide of manganese.

18. A process for the recovery of metallic manganese from manganiferous materials containing phosphorus which comprehends smelting the metalliferous material in the presence of suitable fluxes and carbonaceous reducing agents whilst employing acid furnace practice and temperatures that are high enough to cause extraction of phosphorus with a portion of the iron and low enough to be unfavorable to the reduction of the oxide of manganese whereby a slag containing manganese, but little phosphorus, and only a portion of the iron is obtained.

19. A process for the recovery of metallic manganese from manganiferous materials containing phosphorus which comprehends

- (1) smelting the metalliferous material in the presence of suitable fluxes and carbonaceous reducing agents whilst employing acid furnace practice and temperatures that are high enough to cause extraction of phosphorous with a portion of the iron and low enough to be unfavorable to the reduction of the oxide of manganese whereby a slag containing manganese, but little phosphorous, and only a portion of the iron is provided; and (2) employing the manganiferous slag as the reducible material in the production of the specified alloys as set forth in claim 3 whereby a rich manganese-iron-silicon alloy and a demetallized final slag are produced.
20. A process for the recovery of metallic manganese from manganiferous materials containing phosphorous which comprehends (1) smelting the metalliferous material in the presence of suitable fluxes and carbonaceous reducing agents whilst employing acid furnace practice and temperatures that are high enough to cause extraction of phosphorous with a portion of the iron and low enough to be unfavorable to the reduction of the oxide of manganese whereby a slag containing manganese, but little phosphorous, and only a portion of the iron is provided; and (2) employing the manganiferous slag as the reducible material in the production of the specified alloys as set forth in claim 3 whereby a rich manganese-iron-silicon alloy and a demetallized final slag are produced; and (3) subjecting the pig or cast iron produced in stage (1) to basic purifying treatment whereby carbon steel and a highly phosphorated slag are produced.
21. A cyclic process of manufacturing the specified alloys which comprises the steps of utilizing one of the specified alloys as a reducing agent in a smelting process to produce a metalliferous slag and a substantially pure metallic accessory product, and treating the metalliferous slag as set forth in claim 3 to produce one of the specified alloys.
22. A cyclic process of manufacturing the specified alloys which comprises the steps of utilizing one of the specified alloys as a reducing agent in a smelting process in the presence of a steel bath under conditions whereby an alloy element is added to the liquid steel, to produce a metalliferous slag and a substantially pure metallic product comprising a richly alloyed steel, and treating the metalliferous slag as set forth in claim 3 to produce one of the specified alloys.
23. A cyclic process of manufacturing the specified alloys which comprises smelting matter comprising an oxide of a non-ferrous metal with one of the specified alloys as a reducing agent to produce a metalliferous slag and a substantially pure metallic accessory product, and treating the metalliferous
- slag as set forth in claim 3 to produce one of the specified alloys.
24. A process as set forth in claim 1 wherein the alloy produced contains more than 9% of any number of the metalloids silicon, titanium, and zirconium. 70
25. A process as set forth in claim 1 wherein the alloy produced contains more than 9% of any number of the metalloids silicon, titanium, and zirconium, and wherein independent thermal energy is applied to the furnace charge. 75
- ROBERT WICKERSHAM STIMSON.  
W. BORCHERS.
- 80
- 85
- 90
- 95
- 100
- 105
- 110
- 115
- 120
- 125
- 130